

# UNITED STATES PATENT OFFICE.

GUIDO BLENIO, OF NEW YORK, N. Y., ASSIGNOR TO BLENIO PRODUCTS CORPORATION,  
OF NEW YORK, N. Y., A CORPORATION OF DELAWARE.

## FIREPROOFING SOLUTION.

1,382,618.

Specification of Letters Patent. Patented June 28, 1921.

No Drawing. Application filed January 11, 1919, Serial No. 270,716. Renewed November 18, 1920.  
Serial No. 425,031.

*To all whom it may concern:*

Be it known that I, GUIDO BLENIO, a citizen of the United States, residing at New York, in the county of New York, State of New York, have invented certain new and useful Improvements in Fireproofing Solutions, of which the following is a description.

My invention relates to fire proofing solutions for treating fabrics, wood, or other fibrous materials to render them proof against fire, and has for its object to provide a solution for this purpose which will be effective to render the material treated flame and glow proof without injury to the material, even delicate fabrics, as regards tensile strength or as regards the colors with which the fabric or other material may be dyed or printed, and will at the same time be inexpensive and easily applied.

With these and other objects hereinafter explained in view my invention consists in the solution hereinafter described and claimed.

In preparing my solution for use on fabrics I take 100 gallons of water and dissolve in it 15 pounds of boracic acid crystals, when this is thoroughly dissolved I add to the solution from 5 to 10 gallons of sulfuric acid, depending on the strength of the acid, and then add one half gallon of phosphoric acid. When these ingredients are thoroughly mixed and dissolved I add strong ammonia sufficient to render the solution neutral, it being necessary to the successful use of the solution that it be absolutely neutral as any excess either of acid or alkali will tend to affect colors of fabrics treated or their tensile strength or both.

To this solution I find it desirable, though not essential, to add a small quantity of either gum arabic or tapioca. If gum arabic is used I take for the amount of solution above described from one to five pounds of the gum arabic dissolved in water. If tapioca is used I take the dry tapioca in the proportion of one half ounce to each two gallons of the solution, dissolve it in cold water and cook it thoroughly and add the cooked mass to the solution.

To the solution thus formed I add such amount of water as may be necessary to reduce it to a specific gravity of 12 Baumé.

This forms a stock solution. For use I take from this solution such amount as may be necessary for the amount of fabric to be treated and add sufficient water to reduce the specific gravity to 8 Baumé for delicate fabrics such as lace curtains, cheese cloth or like material. For heavier fabrics less dilution is necessary. The solution if formed of pure materials and made absolutely neutral as above explained will not injure fabrics either as regards tensile strength or color and will render them not only flame proof but also glow proof.

The stock solution above described is effective for fire proofing wood to which it may be applied in any of the usual methods of impregnating wood with fire-proofing or preservative solutions which will cause it to be absorbed by the pores of the wood. But for fire-proofing wood I prefer to use a larger amount of boracic acid than above described and may use from 15 to 25 pounds of the boracic acid crystals instead of the 15 pounds. The solution is, however, to be rendered neutral with strong ammonia. It need not be diluted below 15 Baumé for the stock solution. For use it may be diluted as desired preferably not below 8 Baumé. This solution with the additional amount of boracic acid may be used on fabrics with satisfactory results but the larger amount of boracic acid which is desirable for fire-proofing wood to counteract any hygroscopic tendency of the sulfuric acid but is not necessary for use on fabrics. It is, however, desirable in the solution for use in fire-proofing wood to add the gum arabic or tapioca, preferably the tapioca.

It will, of course, be understood that amounts of the several ingredients may be varied somewhat, the above statement of amounts being approximate only. The neutralization of the solution is essential and in making the solution careful tests should be made to determine this. It is also important to bring the solution to the specific gravity stated or substantially to such specific gravity.

If it is desired to fire-proof wood in connection with electrical apparatus where the wood is required to be as near non-conductive as possible, the sulfuric acid may be

omitted, the amount of phosphoric acid being increased to from 5 to 10 gallons to 100 gallons of water, the amount of boracic acid crystals used being from 20 to 25 pounds.

- 5 This solution should be neutralized with ammonia as before described.

While I prefer to make the stock solution of a specific gravity of 12 Baumé as above stated, it may, for the purposes of transportation to avoid unnecessary amount of water, be made of much higher specific gravity say 20 Baumé or even 25 Baumé. This stronger solution should, on receipt at place at which it is to be used, be reduced 10 to 12 Baumé by the addition of the necessary amount of water.

Any of the fire-proofing solutions above described when rendered absolutely neutral as described, particularly if not of a specific 20 gravity of over 12 Baumé, may be used without injury to the hands of workmen. It is also antiseptic.

Having thus described my invention what I claim is:

- 25 1. A solution for fireproofing resulting from a mixture of sulfuric acid, boracic acid

and phosphoric acid with just sufficient ammonia to render the solution neutral.

2. A solution for fireproofing resulting from a mixture of sulfuric acid, boracic acid, 30 phosphoric acid and tapioca with just sufficient ammonia to render the solution neutral.

3. A solution for fireproofing resulting from a mixture of sulfuric acid, boracic acid, phosphoric acid and tapioca with just sufficient 35 ammonia to render the solution neutral and sufficient water to bring the solution to a specific gravity of 12 Baumé.

4. A solution for fireproofing resulting from a mixture of the following ingredients 40 in substantially the following proportions:

|                                                          |              |
|----------------------------------------------------------|--------------|
| Sulfuric acid                                            | 5 gallons.   |
| Boracic acid crystals                                    | 15 pounds.   |
| Phosphoric acid                                          | 10 gallons.  |
| Water                                                    | 100 gallons. |
| Ammonia: Just sufficient to render the solution neutral. |              |

In testimony whereof I affix my signature this 10th day of January, 1919.

GUIDO BLENIO.